



US008012908B2

(12) **United States Patent**  
**Koide et al.**

(10) **Patent No.:** **US 8,012,908 B2**  
(45) **Date of Patent:** **\*Sep. 6, 2011**

(54) **HEAT-SENSITIVE TRANSFER  
IMAGE-RECEIVING SHEET AND METHOD  
OF PRODUCING IMAGE**

(75) Inventors: **Tomoyuki Koide**, Minami-ashigara (JP);  
**Kazuaki Oguma**, Minami-ashigara (JP);  
**Takuya Arai**, Minami-ashigara (JP)

(73) Assignee: **FUJIFILM Corporation**, Tokyo (JP)

(\*) Notice: Subject to any disclaimer, the term of this patent is extended or adjusted under 35 U.S.C. 154(b) by 1017 days.

This patent is subject to a terminal disclaimer.

(21) Appl. No.: **11/727,012**

(22) Filed: **Mar. 23, 2007**

(65) **Prior Publication Data**

US 2007/0225166 A1 Sep. 27, 2007

(30) **Foreign Application Priority Data**

Mar. 24, 2006 (JP) ..... 2006-083109

(51) **Int. Cl.**

**B41M 5/035** (2006.01)  
**B41M 5/50** (2006.01)

(52) **U.S. Cl.** ..... **503/227; 428/32.39; 428/32.5**

(58) **Field of Classification Search** ..... None  
See application file for complete search history.

(56)

**References Cited**

**U.S. PATENT DOCUMENTS**

7,381,685 B2 \* 6/2008 Oguma et al. ..... 503/227  
7,485,402 B2 \* 2/2009 Arai et al. ..... 430/201

**FOREIGN PATENT DOCUMENTS**

|    |               |         |
|----|---------------|---------|
| JP | 2-25393 A     | 1/1990  |
| JP | 2-89690       | 3/1990  |
| JP | 3-86590 A     | 4/1991  |
| JP | 4-107548 A    | 4/1992  |
| JP | 4-336286 A    | 11/1992 |
| JP | 5-193256      | 8/1993  |
| JP | 5-229289      | 9/1993  |
| JP | 7-17149 A     | 1/1995  |
| JP | 9-131972      | 5/1997  |
| JP | 11-227345 A   | 8/1999  |
| JP | 11-321128     | 11/1999 |
| JP | 2000-238440 A | 9/2000  |
| JP | 2005-335115 A | 12/2005 |

\* cited by examiner

*Primary Examiner* — Bruce H Hess

(74) *Attorney, Agent, or Firm* — Sughrue Mion, PLLC

(57) **ABSTRACT**

A heat-sensitive transfer image-receiving sheet, which is used in an image formation system that continuously produces printed outputs at intervals of 5 seconds or below between the end of ejection of one sheet printed and the start of ejection of the next sheet printed, and which has on a support at least one receptor layer containing a latex polymer comprising repeating units of vinyl chloride component and at least one heat insulation layer containing hollow polymer particles; and a method of forming an image, which uses utilizes the above heat-sensitive image-receiving sheet.

**10 Claims, No Drawings**

## 1

**HEAT-SENSITIVE TRANSFER  
IMAGE-RECEIVING SHEET AND METHOD  
OF PRODUCING IMAGE**

**FIELD OF THE INVENTION**

The present invention relates to a heat-sensitive transfer image-receiving sheet and a method of forming an image. In particular, the present invention relates to a heat-sensitive transfer image-receiving sheet that is suited for high-speed printing and a method of forming an image utilizing the sheet.

**BACKGROUND OF THE INVENTION**

Various heat transfer recording methods have been known so far. Among these methods, dye diffusion transfer recording systems attract attention as a process that can produce a color hard copy having an image quality closest to that of silver salt photography (see, for example, "Joho Kiroku (Hard Copy) to Sono Zairyō no Shintenka (Information Recording (Hard Copy) and New Development of Recording Materials)" published by Toray Research Center Inc., 1993, pp. 241-285; and "Printer Zairyō no Kaihatsu (Development of Printer Materials)" published by CMC Publishing Co., Ltd., 1995, p. 180). Moreover, this system has advantages over silver salt photography: it is a dry system, it enables direct visualization from digital data, it makes reproduction simple, and the like.

In this dye diffusion transfer recording system, a heat-sensitive transfer sheet (hereinafter also referred to as an ink sheet) containing dyes is superposed on a heat-sensitive transfer image-receiving sheet (hereinafter also referred to as an image-receiving sheet), and then the ink sheet is heated by a thermal head whose exothermic action is controlled by electric signals, in order to transfer the dyes contained in the ink sheet to the image-receiving sheet, thereby recording an image information. Three colors: cyan, magenta, and yellow, are used for recording a color image by overlapping one color to other, thereby enabling transferring and recording a color image having continuous gradation for color densities.

In an image-receiving sheet on this system, a receptor layer for fixation of dyes transferred to the sheet is formed on a support, and besides, a layer having high cushion properties, such as a foam layer made up of a resin and a foaming agent or a porous layer containing hollow polymer particles, is generally formed between the support and the receptor layer with the intention of enhancing adhesion of the image-receiving sheet to a transfer sheet (see, e.g., JP-A-11-321128 ("JP-A" means unexamined published Japanese patent application) and JP-A-2-89690).

JP-A-11-321128 discloses forming an intermediate layer containing hollow particles and a high molecular weight compound having resistance to organic solvent as main components on a support by coating and drying, and subsequently forming a receptor layer by applying a resin coating solution prepared using an organic solvent. Herein, the organic-solvent-resistant high-molecular-weight compound used in the intermediate layer plays a role in preventing the hollow particles used in the intermediate layer from being dissolved by the organic solvent used in the receptor layer. However, the formation of a receptor layer by use of a coating solution of resin in an organic solvent has problems that the sensitivity is insufficient and the cost is high, and it has also been desired to introduce improvements in image defects and densities of transferred-ink images.

Further, the heat-sensitive transfer image-receiving sheet disclosed in JP-A-2-89690 includes a hollow-spherical-pigment-dispersed layer and an image-receiving layer (a recep-

## 2

tor layer), but it has a problem that the images after image transfer become blurred. In addition, the cases of using vinyl chloride-series copolymers in receptor layers are disclosed in JP-A-5-193256, JP-A-5-229289, and JP-A-9-131972, but these receptor layers have also been desired to undergo further improvements in view of recent market requirements for rapid processing.

**SUMMARY OF THE INVENTION**

The present invention resides in a heat-sensitive transfer image-receiving sheet, which is used in an image formation system that continuously produces printed outputs at intervals of 5 seconds or below between the end of ejection of one sheet printed and the start of ejection of the next sheet printed, and which has on a support at least one receptor layer containing a latex polymer comprising repeating units of vinyl chloride component and at least one heat insulation layer containing hollow polymer particles.

Further, the present invention resides in a method of forming an image, which method uses:

a heat-sensitive transfer image-receiving sheet which has, on a support, at least one receptor layer containing a latex polymer comprising repeating units of vinyl chloride component and at least one heat insulation layer containing hollow polymer particles, and

a heat-sensitive transfer sheet which has a transfer layer containing a thermally transferable color material; which method comprises the steps of:

superposing the heat-sensitive transfer image-receiving sheet upon the heat-sensitive transfer sheet, so that the transfer layer of the heat-sensitive transfer sheet and the receptor layer of the heat-sensitive transfer image-receiving sheet are brought into face-to-face contact with each other, and

applying a thermal energy according to image signals thereto from a thermal head, and

continuously producing printed outputs on the thermal transfer image-receiving sheets at intervals of 5 seconds or below between the end of ejection of one sheet printed and the start of ejection of the next sheet printed.

Other and further features and advantages of the invention will appear more fully from the following description.

**DETAILED DESCRIPTION OF THE INVENTION**

The present invention provides the following means:

(1) A heat-sensitive transfer image-receiving sheet, which is used in an image formation system that continuously produces printed outputs at intervals of 5 seconds or below between the end of ejection of one sheet printed and the start of ejection of the next sheet printed, and which has on a support at least one receptor layer containing a latex polymer comprising repeating units of vinyl chloride component and at least one heat insulation layer containing hollow polymer particles.

(2) The heat-sensitive transfer image-receiving sheet as described in (1), wherein the heat insulation layer does not contain any resins having poor resistance to an organic solvent other than the hollow polymer particles.

(3) The heat-sensitive transfer image-receiving sheet as described in (1) or (2), wherein at least one of the receptor layer and the heat insulation layer further contains a water-soluble polymer.

(4) The heat-sensitive transfer image-receiving sheet as described in any of (1) to (3), wherein at least one of the receptor layer containing the water-soluble polymer and the heat insulation layer containing the water-soluble polymer

further contains a compound capable of forming crosslinks between molecules of the water-soluble polymer and the compound brings a part or all of the water-soluble polymer molecules into being crosslinked.

(5) A method of forming an image, which method uses:

a heat-sensitive transfer image-receiving sheet which has, on a support, at least one receptor layer containing a latex polymer comprising repeating units of vinyl chloride component and at least one heat insulation layer containing hollow polymer particles, and

a heat-sensitive transfer sheet which has a transfer layer containing a thermally transferable color material (colorant); which method comprises the steps of:

superposing the heat-sensitive transfer image-receiving sheet upon the heat-sensitive transfer sheet, so that the transfer layer of the heat-sensitive transfer sheet and the receptor layer of the heat-sensitive transfer image-receiving sheet are brought into face-to-face contact with each other, and

applying a thermal energy according to image signals thereto from a thermal head, and

continuously producing printed outputs on the thermal transfer image-receiving sheets at intervals of 5 seconds or below between the end of ejection of one sheet printed and the start of ejection of the next sheet printed.

(6) The method of forming an image as described in (5), wherein the heat insulation layer does not contain any resins having poor resistance to an organic solvent other than the hollow polymer particles.

(7) The method of forming an image as described in (5) or (6), wherein at least one of the receptor layer and the heat insulation layer further contains a water-soluble polymer.

(8) The method of forming an image as described in any of (5) to (7), wherein at least one of the receptor layer containing the water-soluble polymer and the heat insulation layer containing the water-soluble polymer further contains a compound capable of forming crosslinks between molecules of the water-soluble polymer and the compound brings a part or all of the water-soluble polymer molecules into being crosslinked.

The present invention will be explained in detail below.

The heat-sensitive transfer image-receiving sheet of the present invention is preferably provided with at least one dye-receiving layer (receptor layer) on a support, and at least one heat insulation layer (porous layer) between the support and the receptor layer. Moreover, an undercoat layer such as a white-background-control layer, a charge-control layer (an electrification-control layer), an adhesive layer, and a primer layer, may be provided between the receptor layer and the heat insulation layer.

The receptor layer and the heat insulation layer are preferably formed by a simultaneous multi-layer coating. When the undercoat layer is provided, the receptor layer, the undercoat layer, and the heat insulation layer may be formed by the simultaneous multi-layer coating.

It is preferable that a curling control layer, a writing layer, and a charge-control layer be formed on the back side of the support. Each layer on the back side of the support can be applied using a usual method such as a roll coating, a bar coating, a gravure coating, and a gravure reverse coating. (Receptor Layer)

The receptor layer performs functions of receiving dyes transferred from an ink sheet and retaining images formed. In the image-receiving sheet according to the present invention, the receptor layer contains a latex polymer. The receptor layer

may be a single layer or multi layers. The receptor layer preferably contains a water-soluble polymer as described later.

<Latex Polymer>

5 The latex polymer for use in the present invention will be explained below.

In the heat-sensitive (thermal) transfer image-receiving sheet of the invention, the latex polymer for use in the receptor layer is a latex of a polymer comprising repeating units of 10 vinyl chloride component and is a dispersion of fine globules of a hydrophobic polymer having water-insoluble vinyl chloride as a monomer unit in a water-soluble dispersion medium. The dispersed state may be one in which polymer is emulsified in a dispersion medium, one in which polymer underwent emulsion polymerization, one in which polymer underwent micelle dispersion, one in which polymer molecules partially have a hydrophilic structure and thus the molecular chains themselves are dispersed in a molecular state, or the like. Latex polymers are described in "Gosei Jushi Emulsion (Synthetic Resin Emulsion)", compiled by Taira Okuda and Hiroshi Inagaki, issued by Kobunshi Kanko Kai (1978); "Gosei Latex no Oyo (Application of Synthetic Latex)", compiled by Takaaki Sugimura, Yasuo Kataoka, Souichi Suzuki, and Keishi Kasahara, issued by Kobunshi Kanko Kai (1993); 25 Soichi Muroi, "Gosei Latex no Kagaku (Chemistry of Synthetic Latex)", issued by Kobunshi Kanko Kai (1970); Yoshiaki Miyosawa (supervisor), "Susei Coating-Zairyō no Kaihatsu to Oyo (Development and Application of Aqueous Coating Material)", issued by CMC Publishing Co., Ltd. 30 (2004) and JP-A-64-538, and so forth. The dispersed particles preferably have a mean particle size (diameter) of about 1 to 50,000 nm, more preferably about 5 to 1,000 nm.

The particle size distribution of the dispersed particles is not particularly limited, and the particles may have either 35 wide particle-size distribution or monodispersed particle-size distribution.

The latex polymer for use in the present invention may be latex of the so-called core/shell type, other than ordinary latex polymer of a uniform structure. When using a core/shell type 40 latex polymer, it is preferred in some cases that the core and the shell have different glass transition temperatures. The glass transition temperature (Tg) of the latex polymer for use in the present invention is preferably -30°C. to 100°C., more preferably 0°C. to 80°C., further more preferably 10°C. to 70°C., and especially preferably 15°C. to 60°C.

As a preferable embodiment of the latex polymer for use in the receptor layer of the image-receiving sheet according to the present invention, there can be preferably used polyvinyl chlorides, a copolymer comprising a vinyl chloride component as a monomer unit (such as a vinyl chloride-vinyl acetate copolymer, and a vinyl chloride-acryl copolymer). In this case, the vinyl chloride monomer unit ratio in the copolymer is preferably in the range of from 50 mol % to 95 mol %. These polymers may be straight-chain, branched, or cross-linked polymers, the so-called homopolymers obtained by polymerizing single type of monomers, or copolymers obtained by polymerizing two or more types of monomers. In the case of the copolymers, these copolymers may be either random copolymers or block copolymers. The molecular weight of each of these polymers is preferably 5,000 to 1,000,000, and further preferably 10,000 to 500,000 in terms of 55 number average molecular weight. Polymers having excessively small molecular weight impart insufficient dynamic strength to the layer containing the latex, and polymers having excessively large molecular weight bring about poor film-forming ability, and therefore both cases are undesirable. Crosslinkable latex polymers are also preferably used.

The latex polymer that can be used in the present invention is commercially available, and polymers described below may be utilized. Examples thereof include G351 and G576 (trade names, manufactured by Nippon Zeon Co., Ltd.); VINYBLAN 240, 270, 277, 375, 386, 609, 550, 601, 602, 630, 660, 671, 683, 680, 680S, 681N, 685R, 277, 380, 381, 410, 430, 432, 860, 863, 865, 867, 900, 900GT, 938, and 950 (trade names, manufactured by Nissin Chemical Industry Co., Ltd.).

These latex polymers may be used singly, or two or more of these polymers may be blended, if necessary.

In the receptor layer of the image-receiving sheet according to the present invention, a ratio of the latex polymer comprising a vinyl chloride component as a monomer unit is preferably 50 mass % or more of the whole solid content in the layer.

In the present invention, it is preferable to prepare the receptor layer by applying an aqueous type coating solution and then drying it. The "aqueous type" so-called here means that 60% by mass or more of the solvent (dispersion medium) of the coating solution is water. As a component other than water in the coating solution, a water miscible organic solvent may be used, such as methyl alcohol, ethyl alcohol, isopropyl alcohol, methyl cellosolve, ethyl cellosolve, dimethylformamide, ethyl acetate, diacetone alcohol, furfuryl alcohol, benzyl alcohol, diethylene glycol monoethyl ether, and oxyethyl phenyl ether.

The latex polymer for use in the present invention preferably has a minimum film-forming temperature (MFT) of from -30 to 90°C., more preferably from 0 to 70°C. In order to control the minimum film-forming temperature, a film-forming aid may be added. The film-forming aid is also called a temporary plasticizer, and it is an organic compound (usually an organic solvent) that reduces the minimum film-forming temperature of a latex polymer. It is described in, for example, Souichi Muroi, "Gosei Latex no Kagaku (Chemistry of Synthetic Latex)", issued by Kobunshi Kanko Kai (1970). Preferable examples of the film-forming aid are listed below, but the compounds that can be used in the present invention are not limited to the following specific examples.

Z-1: Benzyl alcohol

Z-2: 2,2,4-Trimethylpentanediol-1,3-monoisobutyrate

Z-3: 2-Dimethylaminoethanol

Z-4: Diethylene glycol

In combination with the above-described latex polymer for use in the present invention, any polymer can be used. The polymer that can be used in combination is preferably transparent or translucent, and colorless. The polymer may be a natural resin, polymer, or copolymer; a synthetic resin, polymer, or copolymer; or another film-forming medium; and specific examples include gelatins, polyvinyl alcohols, hydroxyethylcelluloses, cellulose acetates, cellulose acetate butyrates, polyvinylpyrrolidones, caseins, starches, polyacrylic acids, polymethylmethacrylic acids, polyvinyl chlorides, polymethacrylic acids, styrene-maleic anhydride copolymers, styrene-acrylonitrile copolymers, styrene-butadiene copolymers, polyvinyl acetals (e.g. polyvinyl formals, polyvinyl butyrals, etc.), polyesters, polyurethanes, phenoxy resins, polyvinylidene chlorides, polyepoxides, polycarbonates, polyvinyl acetates, polyolefins, and polyamides. In the coating liquid, a binder may be dissolved or dispersed in an aqueous solvent or in an organic solvent, or may be in the form of an emulsion.

Examples of a polymer suitably used together with the latex polymer for use in the present invention include polylactic acid esters, polyurethanes, polycarbonates, polyesters,

polyacetals, SBRs, and polyvinyl chlorides. Of these polymers, polyesters, polycarbonates, and polyvinyl chlorides are preferred over the others.

The glass transition temperature (Tg) of the binder for use in the present invention is preferably in the range of -30°C. to 70°C., more preferably -10°C. to 50°C., still more preferably 0°C. to 40°C., in view of film-forming properties (brittleness for working) and image preservability. A blend of two or more types of polymers can be used as the binder.

10 When a blend of two or more polymers is used, the average Tg obtained by summing up the Tg of each polymer weighted by its proportion, is preferably within the foregoing range. Also, when phase separation occurs or when a core-shell structure is adopted, the weighted average Tg is preferably within the foregoing range.

The glass transition temperature (Tg) is calculated according to the following equation:

$$1/Tg = \Sigma (X_i/Tg_i)$$

20 wherein, assuming that the polymer is a copolymer composed of n monomers from i=1 to i=n,  $X_i$  is a weight fraction of the i-th monomer ( $\Sigma X_i = 1$ ) and  $Tg_i$  is glass transition temperature (measured in absolute temperature) of a homopolymer formed from the i-th monomer. The symbol  $\Sigma$  means the sum of i=1 to i=n. The value of the glass transition temperature of a homopolymer formed from each monomer ( $Tg_i$ ) is adopted from J. Brandrup and E. H. Immergut, "Polymer Handbook, 3rd. Edition", Wiley-Interscience (1989).

The polymer used for the binder for use in the present invention can be easily obtained by a solution polymerization method, a suspension polymerization method, an emulsion polymerization method, a dispersion polymerization method, an anionic polymerization method, a cationic polymerization method, or the like. Above all, an emulsion polymerization method in which the polymer is obtained as a latex is the most preferable. Also, a method is preferable in which the polymer is prepared in a solution, and the solution is neutralized or an emulsifier is added to the solution, to which water is then added, to prepare an aqueous dispersion by forced stirring. 30 For example, an emulsion polymerization method comprises conducting polymerization under stirring at about 30°C. to about 100°C. (preferably 60°C. to 90°C.) for 3 to 24 hours by using water or a mixed solvent of water and a water-miscible organic solvent (such as methanol, ethanol, or acetone) as a dispersion medium, a monomer mixture in an amount of 5 mass % to 150 mass % based on the amount of the dispersion medium, an emulsifier and a polymerization initiator. Various conditions such as the dispersion medium, the monomer concentration, the amount of initiator, the amount of emulsifier, the amount of dispersant, the reaction temperature, and the method for adding monomers are suitably determined considering the type of the monomers to be used. Furthermore, it is preferable to use a dispersant when necessary.

55 Generally, the emulsion polymerization method can be conducted according to the disclosures of the following documents: "Gosei Jushi Emarujon (Synthetic Resin Emulsions)" (edited by Taira Okuda and Hiroshi Inagaki and published by Kobunshi Kankokai (1978)); "Gosei Ratekkusu no Oyo (Applications of Synthetic Latexes)" (edited by Takaaki Sugimura, Yasuo Kataoka, Soichi Suzuki, and Keiji Kasahara and published by Kobunshi Kankokai (1993)); and "Gosei Ratekkusu no Kagaku (Chemistry of Synthetic Latexes)" (edited by Soichi Muroi and published by Kobunshi Kankokai (1970)). The emulsion polymerization method for synthesizing the latex polymer for use in the present invention may be a batch polymerization method, a monomer (continuous or

divided) addition method, an emulsion addition method, or a seed polymerization method. The emulsion polymerization method is preferably a batch polymerization method, a monomer (continuous or divided) addition method, or an emulsion addition method in view of the productivity of latex.

The polymerization initiator may be any polymerization initiator having radical generating ability. The polymerization initiator to be used may be selected from inorganic peroxides such as persulfates and hydrogen peroxide, peroxides described in the organic peroxide catalogue of NOF Corporation, and azo compounds as described in the azo polymerization initiator catalogue of Wako Pure Chemical Industries, Ltd. Among them, water-soluble peroxides such as persulfates and water-soluble azo compounds as described in the azo polymerization initiator catalogue of Wako Pure Chemical Industries, Ltd. are preferable; ammonium persulfate, sodium persulfate, potassium persulfate, azobis(2-methylpropionamide) hydrochloride, azobis(2-methyl-N-(2-hydroxyethyl)propionamide), and azobiscyanovaleric acid are more preferable; and peroxides such as ammonium persulfate, sodium persulfate, and potassium persulfate are especially preferable from the viewpoints of image preservability, solubility, and cost.

The amount of the polymerization initiator to be added is, based on the total amount of monomers, preferably 0.3 mass % to 2.0 mass %, more preferably 0.4 mass % to 1.75 mass %, and especially preferably 0.5 mass % to 1.5 mass %.

The polymerization emulsifier to be used may be selected from anionic surfactants, nonionic surfactants, cationic surfactants, and ampholytic surfactants. Among them, anionic surfactants are preferable from the viewpoints of dispersibility and image preservability. Sulfonic acid type anionic surfactants are more preferable because polymerization stability can be ensured even with a small addition amount and they have resistance to hydrolysis. Long chain alkyldiphenyl ether disulfonic acid salts (whose typical example is PELEX SS-H manufactured by Kao Corporation, trade name) are still more preferable, and low electrolyte types such as PIONIN A-43-S (manufactured by Takemoto Oil & Fat Co., Ltd., trade name) are especially preferable.

The amount of sulfonic acid type anionic surfactant as the polymerization emulsifier is preferably 0.1 mass % to 10.0 mass %, more preferably 0.2 mass % to 7.5 mass %, and especially preferably 0.3 mass % to 5.0 mass %, based on the total amount of monomers.

It is preferable to use a chelating agent in synthesizing the latex polymer to be used in the present invention. The chelating agent is a compound capable of coordinating (chelating) a polyvalent ion such as metal ion (e.g., iron ion) or alkaline earth metal ion (e.g., calcium ion), and examples of the chelate compound which can be used include the compounds described in JP-B-6-8956 ("JP-B" means examined Japanese patent publication), U.S. Pat. No. 5,053,322, JP-A-4-73645, JP-A-4-127145, JP-A-4-247073, JP-A-4-305572, JP-A-6-11805, JP-A-5-173312, JP-A-5-66527, JP-A-5-158195, JP-A-6-118580, JP-A-6-110168, JP-A-6-161054, JP-A-6-175299, JP-A-6-214352, JP-A-7-114161, JP-A-7-114154, JP-A-7-120894, JP-A-7-199433, JP-A-7-306504, JP-A-9-43792, JP-A-8-314090, JP-A-10-182571, JP-A-10-182570, and JP-A-11-190892.

Preferred examples of the chelating agent include inorganic chelate compounds (e.g., sodium tripolyphosphate, sodium hexametaphosphate, sodium tetrapolyphosphate), aminopolycarboxylic acid-based chelate compounds (e.g., nitrilotriacetate, ethylenediaminetetraacetate), organic phosphonic acid-based chelate compounds (e.g., compounds described in Research Disclosure, No. 18170, JP-A-52-

102726, JP-A-53-42730, JP-A-56-97347, JP-A-54-121127, JP-A-55-4024, JP-A-55-4025, JP-A-55-29883, JP-A-55-126241, JP-A-55-65955, JP-A-55-65956, JP-A-57-179843, JP-A-54-61125, and West German Patent No. 1045373), 5 polyphenol-based chelating agents, and polyamine-based chelate compounds, with aminopolycarboxylic acid derivatives being particularly preferred.

Preferred examples of the aminopolycarboxylic acid derivative include the compounds shown in the Table attached 10 to "EDTA (-Complexane no Kagaku-) (EDTA-Chemistry of Complexane-)", Nankodo (1977). In these compounds, a part of the carboxyl groups may be substituted by an alkali metal salt such as sodium or potassium or by an ammonium salt. More preferred examples of the aminopolycarboxylic acid derivative include iminodiacetic acid, N-methyliminodiacetic acid, N-(2-aminoethyl)iminodiacetic acid, N-(carbamoylmethyl)imino diacetic acid, nitrilotriacetic acid, ethylenediamine-N,N'-diacetic acid, ethylenediamine-N,N'-di- $\alpha$ -propionic acid, ethylenediamine-N,N'-di- $\beta$ -propionic acid, 15 N,N'-ethylene-bis( $\alpha$ - $\alpha$ -hydroxyphenyl)glycine, N,N'-di(2-hydroxybenzyl)ethylenediamine-N,N'-diacetic acid, ethylenediamine-N,N'-diacetic acid-N,N'-diacetohydroxamic acid, N-hydroxyethylmethylenediamine-N,N',N'-triacetic acid, ethylenediamine-N,N,N',N'-tetraacetic acid, 1,2-propylenediamine-N,N,N',N'-tetraacetic acid, d,1-2,3-diaminobutane-N,N,N',N'-tetraacetic acid, meso-2,3-diaminobutane-N,N,N',N'-tetraacetic acid, 1-phenylethylenediamine-N,N,N',N'-tetraacetic acid, d,1-1,2-diphenylethylenediamine-N,N,N',N'-tetraacetic acid, 26 1,4-diaminobutane-N,N,N',N'-tetraacetic acid, trans-cyclobutane-1,2-diamine-N,N,N',N'-tetraacetic acid, trans-cyclopentane-1,2-diamine-N,N,N',N'-tetraacetic acid, trans-cyclohexane-1,2-diamine-N,N,N',N'-tetraacetic acid, cis-cyclohexane-1,2-diamine-N,N,N',N'-tetraacetic acid, cyclohexane-1,3-diamine-N,N,N',N'-tetraacetic acid, 30 cyclohexane-1,4-diamine-N,N,N',N'-tetraacetic acid, o-phenylenediamine-N,N,N',N'-tetraacetic acid, cis-1,4-diaminobutene-N,N,N',N'-tetraacetic acid, trans-1,4-diaminobutene-N,N,N',N'-tetraacetic acid,  $\alpha$ , $\alpha$ '-diamino-o-xylene-N,N,N',N'-tetraacetic acid, 2-hydroxy-1,3-40 propanediamine-N,N,N',N'-tetraacetic acid, 2,2'-oxy-bis(ethyliminodiacetic acid), 2,2'-ethylenedioxy-bis(ethyliminodiacetic acid), ethylenediamine-N,N'-diacetic acid-N,N'-di- $\alpha$ -propionic acid, ethylenediamine-N,N'-di- $\beta$ -propionic acid, ethylenediamine-N,N,N',N'-tetrapropionic acid, diethylenetriamine-N,N,N',N'',N'''-pentaacetic acid, triethylenetetramine-N,N,N',N'',N'''-hexaacetic acid, and 1,2,3-triaminopropane-N,N,N',N'',N'''-hexaacetic acid. In these compounds, a part of the carboxyl groups may be substituted by an alkali metal salt 45 such as sodium or potassium or by an ammonium salt.

The amount of the chelating agent to be added is preferably 0.01 mass % to 0.4 mass %, more preferably 0.02 mass % to 0.3 mass %, and especially preferably 0.03 mass % to 0.15 mass %, based on the total amount of monomers. When the 55 addition amount of the chelating agent is too small, metal ions entering during the preparation of the latex polymer are not sufficiently trapped, and the stability of the latex against aggregation is lowered, whereby the coating properties become worse. When the amount is too large, the viscosity of the latex increases, whereby the coating properties are lowered.

In the preparation of the latex polymer to be used in the present invention, it is preferable to use a chain transfer agent. As the chain transfer agent, ones described in Polymer Handbook (3rd Edition) (Wiley-Interscience, 1989) are preferable. Sulfur compounds are more preferable because they have high chain-transfer ability and because the required amount is 60

small. Especially, hydrophobic mercaptane-based chain transfer agents such as tert-dodecylmercaptane and n-dodecylmercaptane are preferable.

The amount of the chain transfer agent to be added is preferably 0.2 mass % to 2.0 mass %, more preferably 0.3 mass % to 1.8 mass %, and especially preferably 0.4 mass % to 1.6 mass %, based on the total amount of monomers.

Besides the foregoing compounds, in the emulsion polymerization, use can be made of additives, such as electrolytes, stabilizers, thickeners, defoaming agents, antioxidants, vulcanizers, antifreezing agents, gelling agents, and vulcanization accelerators, as described, for example, in Synthetic Rubber Handbook.

In the coating solution of the latex polymer to be used in the present invention, an aqueous solvent can be used as the solvent, and a water-miscible organic solvent may optionally be used in combination. Examples of the water-miscible organic solvent include alcohols (for example, methyl alcohol, ethyl alcohol, and propyl alcohol), cellosolves (for example, methyl cellosolve, ethyl cellosolve, and butyl cellosolve), ethyl acetate, and dimethylformamide. The amount of the organic solvent to be added is preferably 50 mass % or less of the entire solvent, more preferably 30 mass % or less of the entire solvent.

Furthermore, in the latex polymer to be used in the present invention, the polymer concentration is, based on the amount of the latex liquid, preferably 10 mass % to 70 mass %, more preferably 20 mass % to 60 mass %, and especially preferably 30 mass % to 55 mass %.

The latex polymer in the image-receiving sheet that can be used in the present invention includes a state of a gel or dried film formed by removing a part of solvents by drying after coating.

<Water-Soluble Polymer>

It is preferable that each of the receptor layer and the heat insulation layer (thermal barrier layer), which will be described later, further contains a water-soluble polymer. Herein, the "water-soluble polymer" means a polymer which dissolves, in 100 g water at 20°C., in an amount of preferably 0.05 g or more, more preferably 0.1 g or more, further preferably 0.5 g or more, and particularly preferably 1 g or more. The water-soluble polymer which can be used in the present invention is natural polymers (polysaccharide type, microorganism type, and animal type), semi-synthetic polymers (cellulose-based, starch-based, and alginic acid-based), and synthetic polymer type (vinyl type and others); and synthetic polymers including polyvinyl alcohols, and natural or semi-synthetic polymers using celluloses derived from plant as starting materials, which will be explained later, correspond to the water-soluble polymer usable in the present invention. The latex polymers recited above are not included in the water-soluble polymers which can be used in the present invention.

Among the water-soluble polymers which can be used in the present invention, the natural polymers and the semi-synthetic polymers will be explained in detail. Specific examples include the following polymers: plant type polysaccharides such as gum arabics,  $\kappa$ -carrageenans,  $\iota$ -carrageenans,  $\lambda$ -carrageenans, guar gums (e.g. Supercol, manufactured by Squalon), locust bean gums, pectins, tragacanths, corn starches (e.g. Purity-21, manufactured by National Starch & Chemical Co.), and phosphorylated starches (e.g. National 78-1898, manufactured by National Starch & Chemical Co.); microbial type polysaccharides such as xanthan gums (e.g. Keltrol T, manufactured by Kelco) and dextrans (e.g. Nadex 360, manufactured by National Starch & Chemical Co.); animal type natural polymers such as gelatins (e.g. Crodyne

B419, manufactured by Croda), caseins, sodium chondroitin sulfates (e.g. Cromoist CS, manufactured by Croda); cellulose-based polymers such as ethylcelluloses (e.g. Cellofas WLD, manufactured by I.C.I.), carboxymethylcelluloses (e.g. CMC, manufactured by Daicel), hydroxyethylcelluloses (e.g. HEC, manufactured by Daicel), hydroxypropylcelluloses (e.g. Klucel, manufactured by Aqualon), methylcelluloses (e.g. Viscontran, manufactured by Henkel), nitrocelluloses (e.g. Isopropyl Wet, manufactured by Hercules), and cationated celluloses (e.g. Crodacel QM, manufactured by Croda); starches such as phosphorylated starches (e.g. National 78-1898, manufactured by National Starch & Chemical Co.); alginic acid-based compounds such as sodium alginates (e.g. Keltone, manufactured by Kelco) and propylene glycol alginates; and other polymers such as cationated guar gums (e.g. Hi-care 1000, manufactured by Alcolac) and sodium hyaluronates (e.g. Hyalure, manufactured by Lifecare Biomedical) (all of the names are trade names).

Gelatin is one of preferable embodiments in the present invention. Gelatin having a molecular weight of from 10,000 to 1,000,000 may be used in the present invention. Gelatin that can be used in the present invention may contain an anion such as  $\text{Cl}^-$  and  $\text{SO}_4^{2-}$ , or alternatively a cation such as  $\text{Fe}^{2+}$ ,  $\text{Ca}^{2+}$ ,  $\text{Mg}^{2+}$ ,  $\text{Sn}^{2+}$ , and  $\text{Zn}^{2+}$ . Gelatin is preferably added as an aqueous solution.

Among the water-soluble polymers which can be used in the present invention, the synthetic polymers will be explained in detail. Examples of the acryl type include sodium polyacrylates, polyacrylic acid copolymers, polyacrylamides, polyacrylamide copolymers, and polydiethylaminoethyl(meth)acrylate quaternary salts or their copolymers. Examples of the vinyl type include polyvinylpyrrolidones, polyvinylpyrrolidone copolymers, and polyvinyl alcohols. Examples of the others include polyethylene glycols, polypropylene glycols, polyisopropylacrylamides, polymethyl vinyl ethers, polyethyleneimines, polystyrenesulfonic acids or their copolymers, naphthalenesulfonic acid condensate salts, polyvinylsulfonic acids or their copolymers, polyacrylic acids or their copolymers, acrylic acid or its copolymers, maleic acid copolymers, maleic acid monoester copolymers, acryloylmethylpropanesulfonic acid or its copolymers, polydimethylidiallylammonium chlorides or their copolymers, polyamidines or their copolymers, polyimidazolines, dicyanamide type condensates, epichlorohydrin/dimethylamine condensates, Hofmann decomposed products of polyacrylamides, and water-soluble polyesters (Plascoat Z-221, Z-446, Z-561, Z-450, Z-565, Z-850, Z-3308, RZ-105, RZ-570, Z-730 and RZ-142 (all of these names are trade names), manufactured by Goo Chemical Co., Ltd.).

In addition, highly-water-absorptive polymers, namely, homopolymers of vinyl monomers having  $-\text{COOM}$  or  $-\text{SO}_3\text{M}$  (M represents a hydrogen atom or an alkali metal) or copolymers of these vinyl monomers among them or with other vinyl monomers (for example, sodium methacrylate, ammonium methacrylate, Sumikagel L-5H (trade name) manufactured by Sumitomo Chemical Co., Ltd.) as described in, for example, U.S. Pat. No. 4,960,681 and JP-A-62-245260, may also be used.

Among the water-soluble synthetic polymers usable in the present invention, polyvinyl alcohols will be explained in more detail. Examples of completely saponified polyvinyl alcohol include PVA-105 [polyvinyl alcohol (PVA) content: 94.0 mass % or more; degree of saponification:  $98.5 \pm 0.5$  mol %; content of sodium acetate: 1.5 mass % or less; volatile constituent: 5.0 mass % or less; viscosity (4 mass %; 20°C.):  $5.6 \pm 0.4$  CPS]; PVA-110 [PVA content: 94.0 mass %; degree

## 11

of saponification:  $98.5\pm0.5$  mol %; content of sodium acetate: 1.5 mass %; volatile constituent: 5.0 mass %; viscosity (4 mass %; 20° C.):  $11.0\pm0.8$  CPS]; PVA-117 [PVA content: 94.0 mass %; degree of saponification:  $98.5\pm0.5$  mol %; content of sodium acetate: 1.0 mass %; volatile constituent: 5.0 mass %; viscosity (4 mass %; 20° C.):  $28.0\pm3.0$  CPS]; PVA-117H [PVA content: 93.5 mass %; degree of saponification:  $99.6\pm0.3$  mol %; content of sodium acetate: 1.85 mass %; volatile constituent: 5.0 mass %; viscosity (4 mass %; 20° C.):  $29.0\pm3.0$  CPS]; PVA-120 [PVA content: 94.0 mass %; degree of saponification:  $98.5\pm0.5$  mol %; content of sodium acetate: 1.0 mass %; volatile constituent: 5.0 mass %; viscosity (4 mass %; 20° C.):  $39.5\pm4.5$  CPS]; PVA-124 [PVA content: 94.0 mass %; degree of saponification:  $98.5\pm0.5$  mol %; content of sodium acetate: 1.0 mass %; volatile constituent: 5.0 mass %; viscosity (4 mass %; 20° C.):  $60.0\pm6.0$  CPS]; PVA-124H [PVA content: 93.5 mass %; degree of saponification:  $99.6\pm0.3$  mol %; content of sodium acetate: 1.85 mass %; volatile constituent: 5.0 mass %; viscosity (4 mass %; 20° C.):  $61.0\pm6.0$  CPS]; PVA-CS [PVA content: 94.0 mass %; degree of saponification:  $97.5\pm0.5$  mol %; content of sodium acetate: 1.0 mass %; volatile constituent: 5.0 mass %; viscosity (4 mass %; 20° C.):  $27.5\pm3.0$  CPS]; PVA-CST [PVA content: 94.0 mass %; degree of saponification:  $96.0\pm0.5$  mol %; content of sodium acetate: 1.0 mass %; volatile constituent: 5.0 mass %; viscosity (4 mass %; 20° C.):  $27.0\pm3.0$  CPS]; and PVA-HC [PVA content: 90.0 mass %; degree of saponification: 99.85 mol % or more; content of sodium acetate: 2.5 mass %; volatile constituent: 8.5 mass %; viscosity (4 mass %; 20° C.):  $25.0\pm3.5$  CPS] (all trade names, manufactured by Kuraray Co., Ltd.), and the like.

Examples of partially saponified polyvinyl alcohol include PVA-203 [PVA content: 94.0 mass %; degree of saponification:  $88.0\pm1.5$  mol %; content of sodium acetate: 1.0 mass %; volatile constituent: 5.0 mass %; viscosity (4 mass %; 20° C.):  $3.4\pm0.2$  CPS]; PVA-204 [PVA content: 94.0 mass %; degree of saponification:  $88.0\pm1.5$  mol %; content of sodium acetate: 1.0 mass %; volatile constituent: 5.0 mass %; viscosity (4 mass %; 20° C.):  $3.9\pm0.3$  CPS]; PVA-205 [PVA content: 94.0 mass %; degree of saponification:  $88.0\pm1.5$  mol %; content of sodium acetate: 1.0 mass %; volatile constituent: 5.0 mass %; viscosity (4 mass %; 20° C.):  $5.0\pm0.4$  CPS]; PVA-210 [PVA content: 94.0 mass %; degree of saponification:  $88.0\pm1.0$  mol %; content of sodium acetate: 1.0 mass %; volatile constituent: 5.0 mass %; viscosity (4 mass %; 20° C.):  $9.0\pm1.0$  CPS]; PVA-217 [PVA content: 94.0 mass %; degree of saponification:  $88.0\pm1.0$  mol %; content of sodium acetate: 1.0 mass %; volatile constituent: 5.0 mass %; viscosity (4 mass %; 20° C.):  $22.5\pm2.0$  CPS]; PVA-220 [PVA content: 94.0 mass %; degree of saponification:  $88.0\pm1.0$  mol %; content of sodium acetate: 1.0 mass %; volatile constituent: 5.0 mass %; viscosity (4 mass %; 20° C.):  $30.0\pm3.0$  CPS]; PVA-224 [PVA content: 94.0 mass %; degree of saponification:  $88.0\pm1.5$  mol %; content of sodium acetate: 1.0 mass %; volatile constituent: 5.0 mass %; viscosity (4 mass %; 20° C.):  $44.0\pm4.0$  CPS]; PVA-228 [PVA content: 94.0 mass %; degree of saponification:  $88.0\pm1.5$  mol %; content of sodium acetate: 1.0 mass %; volatile constituent: 5.0 mass %; viscosity (4 mass %; 20° C.):  $65.0\pm5.0$  CPS]; PVA-235 [PVA content: 94.0 mass %; degree of saponification:  $88.0\pm1.5$  mol %; content of sodium acetate: 1.0 mass %; volatile constituent: 5.0 mass %; viscosity (4 mass %; 20° C.):  $95.0\pm15.0$  CPS]; PVA-217EE [PVA content: 94.0 mass %; degree of saponification:  $88.0\pm1.0$  mol %; content of sodium acetate: 1.0 mass %; volatile constituent: 5.0 mass %; viscosity (4 mass %; 20° C.):  $23.0\pm3.0$  CPS]; PVA-217E [PVA

## 12

content: 94.0 mass %; degree of saponification:  $88.0\pm1.0$  mol %; content of sodium acetate: 1.0 mass %; volatile constituent: 5.0 mass %; viscosity (4 mass %; 20° C.):  $23.0\pm3.0$  CPS]; PVA-220E [PVA content: 94.0 mass %; degree of saponification:  $88.0\pm1.0$  mol %; content of sodium acetate: 1.0 mass %; volatile constituent: 5.0 mass %; viscosity (4 mass %; 20° C.):  $31.0\pm4.0$  CPS]; PVA-224E [PVA content: 94.0 mass %; degree of saponification:  $88.0\pm1.0$  mol %; content of sodium acetate: 1.0 mass %; volatile constituent: 5.0 mass %; viscosity (4 mass %; 20° C.):  $45.0\pm5.0$  CPS]; PVA-403 [PVA content: 94.0 mass %; degree of saponification:  $80.0\pm1.5$  mol %; content of sodium acetate: 1.0 mass %; volatile constituent: 5.0 mass %; viscosity (4 mass %; 20° C.):  $3.1\pm0.3$  CPS]; PVA-405 [PVA content: 94.0 mass %; degree of saponification:  $81.5\pm1.5$  mol %; content of sodium acetate: 1.0 mass %; volatile constituent: 5.0 mass %; viscosity (4 mass %; 20° C.):  $4.8\pm0.4$  CPS]; PVA-420 [PVA content: 94.0 mass %; degree of saponification:  $79.5\pm1.5$  mol %; content of sodium acetate: 1.0 mass %; volatile constituent: 5.0 mass %]; PVA-613 [PVA content: 94.0 mass %; degree of saponification:  $93.5\pm1.0$  mol %; content of sodium acetate: 1.0 mass %; volatile constituent: 5.0 mass %; viscosity (4 mass %; 20° C.):  $16.5\pm2.0$  CPS]; L-8 [PVA content: 96.0 mass %; degree of saponification:  $71.0\pm1.5$  mol %; content of sodium acetate: 1.0 mass % (ash); volatile constituent: 3.0 mass %; viscosity (4 mass %; 20° C.):  $5.4\pm0.4$  CPS] (all trade names, manufactured by Kuraray Co., Ltd.), and the like.

The above values were measured in the manner described in JIS K-6726-1977.

With respect to modified polyvinyl alcohols, those described in Koichi Nagano, et al., "Poval", Kobunshi Kankokai, Inc. are useful. The modified polyvinyl alcohols include polyvinyl alcohols modified by cations, anions, —SH compounds, alkylthio compounds, or silanols.

Examples of such modified polyvinyl alcohols (modified PVA) include C polymers such as C-118, C-318, C-318-2A, and C-506 (all being trade names of Kuraray Co., Ltd.); HL polymers such as HL-12E and HL-1203 (all being trade names of Kuraray Co., Ltd.); HM polymers such as HM-03 and HM-N-03 (all being trade names of Kuraray Co., Ltd.); K polymers such as KL-118, KL-318, KL-506, KM-118T, and KM-618 (all being trade names of Kuraray Co., Ltd.); M polymers such as M-115 (a trade name of Kuraray Co., Ltd.); MP polymers such as MP-102, MP-202, and MP-203 (all being trade names of Kuraray Co., Ltd.); MPK polymers such as MPK-1, MPK-2, MPK-3, MPK-4, MPK-5, and MPK-6 (all being trade names of Kuraray Co., Ltd.); R polymers such as R-1130, R-2105, and R-2130 (all being trade names of Kuraray Co., Ltd.); and V polymers such as V-2250 (a trade name of Kuraray Co., Ltd.).

The viscosity of polyvinyl alcohol can be adjusted or stabilized by adding a trace amount of a solvent or an inorganic salt to an aqueous solution of polyvinyl alcohol, and there can be employed compounds described in the aforementioned reference "Poval", Koichi Nagano et al., published by Kobunshi Kankokai, pp. 144-154. For example, a coated-surface quality can be improved by an addition of boric acid. The amount of boric acid added is preferably 0.01 to 40 mass % with respect to polyvinyl alcohol.

Preferred binders are transparent or semitransparent, generally colorless, and water-soluble. Examples include natural resins, polymers and copolymers; synthetic resins, polymers, and copolymers; and other media that form films: for example, rubbers, polyvinyl alcohols, hydroxyethyl celluloses, cellulose acetates, cellulose acetate butylates, polyvinylpyrrolidones, starches, polyacrylic acids, polymethyl methacrylates, polyvinyl chlorides, polymethacrylic acids, styrene/maleic acid anhydride copolymers, styrene/acryloni-

trile copolymers, styrene/butadiene copolymers, polyvinylacetals (e.g., polyvinylformals and polyvinylbutyral), polyesters, polyurethanes, phenoxy resins, polyvinylidene chlorides, polyepoxides, polycarbonates, polyvinyl acetates, polyolefins, cellulose esters, and polyamides.

The amount of the water-soluble polymer added to the receptor layer is preferably from 1 to 25% by mass, more preferably from 1 to 10% by mass based on the total mass of the receptor layer.

<Crosslinking Agent>

It is preferable that the above-mentioned water-soluble polymer contained in the receptor layer is partly or entirely crosslinked with a crosslinking agent.

The crosslinking agent is required to have a plurality of groups capable of reacting with an amino group, a carboxyl group, a hydroxyl group, or the like, but the agent to be used may be suitably selected depending on the kind of the water-soluble polymer. Thus, there is no particular limitation for the kind of the crosslinking agent. It is suitable to use each of methods described in T. H. James; "THE THEORY OF THE PHOTOGRAPHIC PROCESS FOURTH EDITION", published by Macmillan Publishing Co., Inc. (1977), pp. 77-87, and crosslinking agents described in, for example, U.S. Pat. No. 4,678,739, col. 41; JP-A-59-116655, JP-A-62-245261, and JP-A-61-18942. Both crosslinking agents of an inorganic compound (e.g., chrome alum, boric acid and salts thereof) and crosslinking agents of an organic compound may be preferably used. Alternatively, the crosslinking agent to be used may be a mixture solution containing a chelating agent and a zirconium compound, whose pH is in the range of 1 to 7, as described in JP-A-2003-231775.

Specific examples of the crosslinking agent include epoxy-series compounds (e.g., diglycidyl ethyl ether, ethyleneglycol diglycidyl ether, 1,4-butanediol diglycidyl ether, 1,6-diglycidyl cyclohexane, N,N-diglycidyl-4-glycidyloxyaniline, sorbitol polyglycidyl ether, glycerol polyglycidyl ether, compounds described in JP-A-6-329877, JP-A-7-309954 and the like, and DIC FINE EM-60 (trade name, manufactured by DAINIPPON INK AND CHEMICALS, INCORPORATED)), aldehyde-series compounds (e.g., formaldehyde, glyoxal, glutaldehyde), active halogen-series compounds (e.g., 2,4-dichloro-4-hydroxy-1,3,5-s-triazine, and compounds described in U.S. Pat. No. 3,325,287 and the like), active vinyl-series compounds (e.g., 1,3,5-trisacryloylhexahydro-s-triazine, bisvinylsulfonylmethyl ether, N,N'-ethylene-bis(vinylsulfonylactamido)ethane, and compounds described in JP-B-53-41220, JP-B-53-57257, JP-B-59-162546, JP-B-60-80846 and the like), mucohalogen acid compounds (e.g., mucochloric acid), N-carbamoylpyridinium salt compounds (e.g., (1-morpholinocarbonyl-3-pyridinio)methanesulfonate), haloamidinium salt compounds (e.g., 1-(1-chloro-1-pyridinomethylene)pyrrolidinium, 2-naphthalenesulfonate), N-methylol-series compounds (e.g., dimethylolurea, methyloldimethylhydantoin), carbodiimido compounds (e.g., polycarbodiimido compounds derived from isoholondiisocyanate as described in JP-A-59-187029 and JP-B-5-27450, carbodiimido compounds derived from tetramethylxylylene diisocyanate as described in JP-A-7-330849, multi-branch type carbodiimido compounds described in JP-A-10-30024, carbodiimido compounds derived from dicyclohexylmethane diisocyanate as described in JP-A-2000-7642, and CARBODILITE V-02, V-02-L2, V-04, V-06, E-01 and E-02 (trade names, manufactured by Nisshinbo Industries, Inc.)), oxazoline compounds (e.g., oxazoline compounds described in JP-A-2001-215653 and EPOCRON K-1010E, K-1020E, K-1030E, K-2010E, K-2020E, K-2030E, WS-500 and WS-700 (trade names,

manufactured by NIPPON SHOKUBAI CO., LTD.)), isocyanate compounds (e.g., dispersible isocyanate compounds described in JP-A-7-304841, JP-A-8-277315, JP-A-10-45866, JP-A-9-71720, JP-A-9-328654, JP-A-9-104814, JP-A-2000-194045, JP-A-2000-194237 and JP-A-2003-64149, and Duranate WB40-100, WB40-80D, WT20-100 and WT30-100 (trade names, manufactured by Asahi Kasei Corporation), CR-60N (trade name, manufactured by DAINIPPON INK AND CHEMICALS, INCORPORATED)), polymer (high molecular) hardeners (e.g., compounds described in JP-A-62-234157 and the like); boric acid and salts thereof, borax, and alum.

Preferable compounds as the crosslinking agent include epoxy-series compounds, aldehyde-series compounds, active halogen-series compounds, active vinyl-series compounds, N-carbamoylpyridinium salt compounds, N-methylol-series compounds (e.g., dimethylolurea, methyloldimethylhydantoin), carbodiimido compounds, oxazoline compounds, isocyanate compounds, polymer hardeners (e.g., compounds described in JP-A-62-234157 and the like), boric acid and salts thereof, borax, and alum. More preferable crosslinking agents include epoxy-series compounds, active halogen-series compounds, active vinyl-series compounds, N-carbamoylpyridinium salt compounds, N-methylol-series compounds (e.g., dimethylolurea, methyloldimethylhydantoin), polymer hardeners (e.g., compounds described in JP-A-62-234157 and the like) and boric acid. The above-mentioned crosslinking agent may be used singly or in combination of two or more.

The crosslinking agent that can be used in the present invention may be added to the water-soluble polymer solution in advance, or may be added at the last step for the preparation of the coating solution. Alternatively, the crosslinking agent may be added just before the coating.

The water-soluble polymer in the receptor layer is preferably cross-linked in a ratio of from 0.1 to 20 mass %, more preferably from 1 to 10 mass %, among the entire water-soluble polymer, even though the ratio varies depending on the kind of the crosslinking agent.

The addition amount of the crosslinking agent that can be used in the present invention varies depending on the kinds of the water-soluble binder and the crosslinking agent, but it is preferable that the amount is approximately in the range of from 0.1 to 50 mass parts, more preferably from 0.5 to 20 mass parts, and further more preferably from 1 to 10 mass parts, based on 100 mass parts of the water-soluble polymer contained in the constituting layer.

<Ultraviolet Absorber>

Also, in the present invention, in order to improve light resistance, an ultraviolet absorber may be added to the receptor layer. In this case, when this ultraviolet absorber is made to have a higher molecular weight, it can be secured to the receptor layer so that it can be prevented, for instance, from being diffused into the ink sheet and from being sublimated and vaporized by heating.

As the ultraviolet absorber, compounds having various ultraviolet absorber skeletons, which are widely used in the field of information recording, may be used. Specific examples of the ultraviolet absorber may include compounds having a 2-hydroxybenzotriazole type ultraviolet absorber skeleton, 2-hydroxybenzotriazine type ultraviolet absorber skeleton, or 2-hydroxybenzophenone type ultraviolet absorber skeleton. Compounds having a benzotriazole-type or triazine-type skeleton are preferable from the viewpoint of ultraviolet absorbing ability (absorption coefficient) and stability, and compounds having a benzotriazole-type or benzophenone-type skeleton are preferable from the viewpoint of

obtaining a higher-molecular weight and using in a form of a latex. Specifically, ultraviolet absorbers described in, for example, JP-A-2004-361936 may be used.

The ultraviolet absorber preferably absorbs light at wavelengths in the ultraviolet region, and the absorption edge of the absorption of the ultraviolet absorber is preferably out of the visible region. Specifically, when it is added to the receptor layer to form a heat-sensitive transfer image-receiving sheet, the heat-sensitive transfer image-receiving sheet has a reflection density of, preferably, Abs 0.5 or more at 370 nm, and more preferably Abs 0.5 or more at 380 nm. Also, the heat-sensitive transfer image-receiving sheet has a reflection density of, preferably, Abs 0.1 or less at 400 nm. If the reflection density at a wavelength range exceeding 400 nm is high, it is not preferable because an image is made yellowish.

In the present invention, the ultraviolet absorber is preferably made to have a higher molecular weight. The ultraviolet absorber has a weight average molecular weight of preferably 10,000 or more, and more preferably 100,000 or more. As a means of obtaining a higher-molecular weight ultraviolet absorber, it is preferable to graft an ultraviolet absorber on a polymer. The polymer as the principal chain preferably has a polymer skeleton less capable of being dyed than the receptor polymer to be used together. Also, when the polymer is used to form a film, the film preferably has sufficient film strength. The graft ratio of the ultraviolet absorber to the polymer principal chain is preferably 5 to 20% by mass and more preferably 8 to 15% by mass.

Also, it is more preferable that the ultraviolet-absorber-grafted polymer is made to be used in a form of a latex. When the polymer is made to be used in a form of a latex, an aqueous dispersion-system coating solution may be used in application and coating to form the receptor layer, and this enables reduction of production cost. As a method of making the latex polymer (or making the polymer latex-wise), a method described in, for example, Japanese Patent No. 3,450,339 may be used. As the ultraviolet absorber to be used in a form of a latex, the following commercially available ultraviolet absorbers may be used which include ULS-700, ULS-1700, ULS-1383MA, ULS-1635MH, XL-7016, ULS-933LP, and ULS-935LH, manufactured by Ipposha Oil Industries Co., Ltd.; and New Coat UVA-1025W, New Coat UVA-204W, and New Coat UVA-4512M, manufactured by Shin-Nakamura Chemical Co., Ltd. (all of these names are trade names).

In the case of using an ultraviolet-absorber-grafted polymer in a form of a latex, it may be mixed with a latex of the receptor polymer capable of being dyed, and the resulting mixture is coated. By doing so, a receptor layer, in which the ultraviolet absorber is homogeneously dispersed, can be formed.

The addition amount of the ultraviolet-absorber-grafted polymer or its latex is preferably 5 to 50 parts by mass, and more preferably 10 to 30 parts by mass, to 100 parts by mass of the latex of the receptor polymer capable of being dyed to be used to form the receptor layer.

#### <Emulsified Dispersion>

In the present invention, incorporation of an emulsified dispersion (emulsion) in the receptor layer or the heat insulation layer is preferable, especially when the latex polymer is used.

The term "emulsification" as used herein follows the commonly used definition. According to "Kagaku Daijiten (EN-CYCLOPEDIA CHIMICA)", Kyoritsu Shuppan Co., Ltd., for example, "emulsification" is defined as "a phenomenon in which, in one liquid, another liquid which does not dissolve in the first liquid are dispersed as fine globules, to form an emulsion". In addition, the term "emulsified dispersion"

refers to "a dispersion in which fine globules of one liquid are dispersed in another liquid which does not dissolve the globules". The "emulsified dispersion" preferred in the present invention is "a dispersion of oil globules in water". The content of an emulsified dispersion in the image-receiving sheet of the present invention is preferably from 0.03 g/m<sup>2</sup> to 25.0 g/m<sup>2</sup>, more preferably from 1.0 g/m<sup>2</sup> to 20.0 g/m<sup>2</sup>.

In the present invention, it is preferable that a high-boiling solvent be included as an oil-soluble substance in the emulsified dispersion. Examples of the high-boiling solvent preferably used include phthalic acid esters (such as dibutyl phthalate, diethyl phthalate, and di-2-ethyl-hexyl phthalate), phosphoric or phosphonic acid esters (such as triphenyl phosphate, tricresyl phosphate, tri-2-ethylhexyl phosphate), fatty acid esters (such as di-2-ethylhexyl succinate and tributyl citrate), benzoic acid esters (such as 2-ethylhexyl benzoate and dodecylbenzoate), amides (such as N,N-diethyldecanamide and N,N-dimethyloleinamide), alcohol and phenol compounds (such as isostearyl alcohol and 2,4-di-tert-amylophenol), anilines (such as N,N-dibutyl-2-butoxy-5-tert-octylaniline), chlorinated paraffins, hydrocarbons (such as dodecylbenzene and diisopropylnaphthalene), and carboxylic acids (such as 2-(2, 4-di-tert-amylphenoxy)butyric acid). Of these high-boiling solvents, phosphoric or phosphonic acid esters (such as triphenyl phosphate, tricresyl phosphate, and tri-2-ethylhexyl phosphate) are preferred over the others. In addition to such a high-boiling solvent, an organic solvent having a boiling point of 30° C. to 160° C. (such as ethyl acetate, butyl acetate, methyl ethyl ketone, cyclohexanone, methyl cellosolve acetate, or dimethylformamide) may be used as an auxiliary solvent. The content of high-boiling solvent in the emulsified dispersion is preferably from 3.0 to 25% by mass, and more preferably from 5.0 to 20% by mass.

It is preferable that the emulsified dispersion further contain an agent for imparting fastness to images and an ultraviolet absorbent. The compounds preferably used as such agents are any of the compounds represented by formulae (B), (Ph), (E-1) to (E-3), (TS-I) to (TS-VII), (TS-VIIIA), (UA) to (UE) disclosed in JP-A-2004-361936. Further, homopolymers or copolymers insoluble in water and soluble in organic solvents (preferably the compounds disclosed in JP-A-2004-361936, paragraph Nos. 0208 to 0234) may be included therein.

<Releasing Agent>

Also, a releasing agent may be compounded in the receptor layer, in order to prevent thermal welding with the heat-sensitive transfer sheet at the time of forming an image. As the releasing agent, a silicone oil, a phosphate-based plasticizer, or a fluorine-series compound may be used, and the silicone oil is particularly preferably used. As the silicone oil, modified silicone oil, such as epoxy-modified, alkyl-modified, amino-modified, carboxyl-modified, alcohol-modified, fluorine-modified, alkyl aralkyl polyether-modified, epoxy/polyether-modified, or polyether-modified silicone oil, is preferably used. Among these, a reaction product between vinyl-modified silicone oil and hydrogen-modified silicone oil is preferable. The amount of the releasing agent is preferably 0.2 to 30 parts by mass, to 100 parts by mass of the receptor polymer.

The amount of the receptor layer to be applied is preferably 0.5 to 10 g/m<sup>2</sup> (solid basis, hereinafter, the amount to be applied in the present specification means a value on a solid basis unless otherwise noted). The film thickness of the receptor layer is preferably 1 to 20 μm.

#### (Heat Insulation Layer)

A heat insulation layer serves to protect the support from heat when a thermal head is used to carry out a transfer

operation under heating. Also, because the heat insulation layer has high cushion characteristics, a heat-sensitive transfer image-receiving sheet having high printing sensitivity can be obtained even in the case of using paper as a substrate (support). The heat insulation layer may be a single layer, or multi-layers. The heat insulation layer is arranged at a nearer location to the support than the receptor layer.

In the image-receiving sheet according to the present invention, the heat insulation layer contains hollow polymer particles.

The hollow polymer particles in the present invention are polymer particles having independent pores inside of the particles. Examples of the hollow polymer particles include (1) non-foaming type hollow particles obtained in the following manner: water is contained inside of a capsule wall formed of a polystyrene, acryl resin, or styrene/acryl resin and, after a coating solution is applied and dried, the water in the particles is vaporized out of the particles, with the result that the inside of each particle forms a hollow; (2) foaming type microballoons obtained in the following manner: a low-boiling point liquid such as butane and pentane is encapsulated in a resin constituted of any one of polyvinylidene chloride, polyacrylonitrile, polyacrylic acid and polyacrylate, and their mixture or polymer, and after the resin coating material is applied, it is heated to expand the low-boiling point liquid inside of the particles whereby the inside of each particle is made to be hollow; and (3) microballoons obtained by foaming the above (2) under heating in advance, to make hollow polymer particles.

These hollow polymer particles preferably have a hollow ratio of about 20 to 70%, and may be used in combinations of two or more. Specific examples of the above (1) include Rohpake 1055 manufactured by Rohm and Haas Co.; Boncoat PP-1000 manufactured by Dainippon Ink and Chemicals, Incorporated; SX866(B) manufactured by JSR Corporation; and Nippol MH5055 manufactured by Nippon Zeon (all of these product names are trade names). Specific examples of the above (2) include F-30 and F-50 manufactured by Matsumoto Yushi-Seiyaku Co., Ltd. (all of these product names are trade names). Specific examples of the above (3) include F-30E manufactured by Matsumoto Yushi-Seiyaku Co., Ltd, and Expance 461DE, 551DE and 551DE20 manufactured by Nippon Ferrite (all of these product names are trade names). The hollow polymer particles for use in the heat insulation layer may be a latex thereof.

A water-dispersible resin or water-soluble resin is preferably contained, as a binder, in the heat insulation layer containing the hollow polymer particles. As the binder resin that can be used in the present invention, known resins such as an acryl resin, styrene/acryl copolymer, polystyrene resin, polyvinyl alcohol resin, vinyl acetate resin, ethylene/vinyl acetate copolymer, vinyl chloride/vinyl acetate copolymer, styrene/butadiene copolymer, polyvinylidene chloride resin, cellulose derivative, casein, starch, and gelatin may be used. Also, these resins may be used either singly or as mixtures.

The solid content of the hollow polymer particles in the heat insulation layer preferably falls in a range from 5 to 2,000 parts by mass when the solid content of the binder resin is 100 parts by mass. The solid content of the hollow polymer particles is preferably 50% by mass or more, more preferably 60% by mass or more, and further preferably 60% by mass or more, based on the total solid content of the hollow polymer particles and the binder resin. Also, the ratio by mass of the solid content of the hollow polymer particles in the coating solution is preferably 1 to 70% by mass and more preferably 10 to 40% by mass. If the ratio of the hollow polymer particles is excessively low, sufficient heat insulation cannot be

obtained, whereas if the ratio of the hollow polymer particles is excessively large, the adhesion between the hollow polymers particles is reduced, posing problems, for example, powder fall or film separation.

5 The particle size of the hollow polymer particles is preferably 0.1 to 20  $\mu\text{m}$ , more preferably 0.1 to 2  $\mu\text{m}$  and particularly preferably 0.1 to 1  $\mu\text{m}$ . Also, the glass transition temperature (Tg) of the hollow polymer particles is preferably 70°C. or more and more preferably 100°C. or more.

10 It is preferable that the image-receiving sheet of the present invention do not contain, in the heat insulation layer, an aqueous dispersion of a resin having poor resistance to an organic solvent, other than the hollow polymer particles. Incorporation of the resin having poor resistance to an organic

15 solvent (resin having a dye-dyeing affinity or a resin capable of being dyed) in the heat insulation layer is not preferable in view of increase in loss of image definition (i.e. increase in blurring) after image transfer. It is assumed that the color-edge definition loss (image blurring) increases by the reason

20 that owing to the presence of both the resin having a dye-dyeing affinity and the hollow polymer particles in the heat insulation layer, a transferred dye that has dyed the receptor layer migrates through the heat insulation layer adjacent thereto at the lapse of time.

25 Herein, the term "poor resistance to an organic solvent" means that a solubility in an organic solvent (e.g., methyl ethyl ketone, ethyl acetate, benzene, toluene, xylene) is 1 mass % or more, preferably 0.5 mass % or more. For example, the above-mentioned latex polymer is included in the category of the resin having "poor resistance to an organic solvent".

30 The heat insulation layer preferably contains the above-mentioned water-soluble polymer. Preferable compounds of the water-soluble polymer are the same as mentioned above.

35 The amount of the water-soluble polymer to be added in the heat insulation layer is preferably from 1 to 75 mass %, more preferably from 1 to 50 mass % of the entire mass of the heat insulation layer.

40 The heat insulation layer preferably contains a gelatin. The amount of the gelatin in the coating solution for the heat insulation layer is preferably 0.5 to 14% by mass, and particularly preferably 1 to 6% by mass. Also, the coating amount of the above hollow polymer particles in the heat insulation layer is preferably 1 to 100  $\text{g/m}^2$ , and more preferably 5 to 20  $\text{g/m}^2$ .

45 The water-soluble polymer that is contained in the heat insulation layer is preferably cross-linked with a crosslinking agent. Preferable compounds as well as a preferable amount of the crosslinking agent to be used are the same as mentioned above.

50 A preferred ratio of a cross-linked water-soluble polymer in the heat insulation layer varies depending on the kind of the crosslinking agent, but the water-soluble polymer in the heat insulation layer is crosslinked by preferably 0.1 to 20 mass %, more preferably 1 to 10 mass %, based on the entire water-soluble polymer.

55 A thickness of the heat insulation layer containing the hollow polymer particles is preferably from 5 to 50  $\mu\text{m}$ , more preferably from 5 to 40  $\mu\text{m}$ .

60 (Undercoat Layer)

An undercoat layer may be formed between the receptor layer and the heat insulation layer. As the undercoat layer, for example, a white background regulation layer, a charge regulation layer, an adhesive layer or a primer layer is formed.

65 These layers may be formed in the same manner as those described in, for example, each specification of Japanese Patent Nos. 3,585,599 and 2,925,244.

(Support)

In the present invention, a waterproof support is preferably used as the support. The use of the waterproof support makes it possible to prevent the support from absorbing moisture, whereby a fluctuation in the performance of the receptor layer with lapse of time can be prevented. As the waterproof support, for example, coated paper or laminate paper may be used.

Coated Paper

The coated paper is paper obtained by coating a sheet such as base paper with various resins, rubber latexes, or high-molecular materials, on one side or both sides of the sheet, wherein the coating amount differs depending on its use. Examples of such coated paper include art paper, cast coated paper, and Yankee paper.

It is proper to use a thermoplastic resin as the resin to be applied to the surface(s) of the base paper. As such a thermoplastic resin, the following thermoplastic resins (A) to (H) may be exemplified.

(A) Polyolefin resins such as polyethylene resin and polypropylene resin; copolymer resins composed of an olefin such as ethylene or propylene and another vinyl monomer; and acrylic resin.

(B) Thermoplastic resins having an ester linkage: for example, polyester resins obtained by condensation of a dicarboxylic acid component (such a dicarboxylic acid component may be substituted with a sulfonic acid group, a carboxyl group, or the like) and an alcohol component (such an alcohol component may be substituted with a hydroxyl group, or the like); polyacrylate resins or polymethacrylate resins such as polymethylmethacrylate, polybutylmethacrylate, polymethylacrylate, polybutylacrylate, or the like; polycarbonate resins, polyvinyl acetate resins, styrene acrylate resins, styrene-methacrylate copolymer resins, vinyltoluene acrylate resins, or the like.

Concrete examples of them are those described in JP-A-59-101395, JP-A-63-7971, JP-A-63-7972, JP-A-63-7973, and JP-A-60-294862.

Commercially available thermoplastic resins usable herein are, for example, Vylon 290, Vylon 200, Vylon 280, Vylon 300, Vylon 103, Vylon GK-140, and Vylon GK-130 (products of Toyobo Co., Ltd.); Tafton NE-382, Tafton U-5, ATR-2009, and ATR-2010 (products of Kao Corporation); Elitel UE 3500, UE 3210, XA-8153, KZA-7049, and KZA-1449 (products of Unitika Ltd.); and Polyester TP-220 and R-188 (products of The Nippon Synthetic Chemical Industry Co., Ltd.); and thermoplastic resins in the Hyros series from Seiko Chemical Industries Co., Ltd., and the like (all of these names are trade names).

(C) Polyurethane resins, etc.

(D) Polyamide resins, urea resins, etc.

(E) Polysulfone resins, etc.

(F) Polyvinyl chloride resins, polyvinylidene chloride resins, vinyl chloride/vinyl acetate copolymer resins, vinyl chloride/vinyl propionate copolymer resins, etc.

(G) Polyol resins such as polyvinyl butyral; and cellulose resins such as ethyl cellulose resin and cellulose acetate resin, and

(H) Polycaprolactone resins, styrene/maleic anhydride resins, polyacrylonitrile resins, polyether resins, epoxy resins, and phenolic resins.

The thermoplastic resins may be used either alone or in combination of two or more.

The thermoplastic resin may contain a whitener, a conductive agent, a filler, a pigment or dye including, for example, titanium oxide, ultramarine blue, and carbon black; or the like, if necessary.

Laminated Paper

The laminated paper is a paper which is formed by laminating various kinds of resin, rubber, polymer sheets or films on a sheet such as a base paper or the like. Specific examples of the materials useable for the lamination include polyolefins, polyvinyl chlorides, polyethylene terephthalates, polystyrenes, polymethacrylates, polycarbonates, polyimides, and triacetylcelluloses. These resins may be used alone, or in combination of two or more.

Generally, the polyolefins are prepared by using a low-density polyethylene. However, for improving the thermal resistance of the support, it is preferred to use a polypropylene, a blend of a polypropylene and a polyethylene, a high-density polyethylene, or a blend of a high-density polyethylene and a low-density polyethylene. From the viewpoint of cost and its suitableness for the laminate, it is preferred to use the blend of a high-density polyethylene and a low-density polyethylene.

The blend of a high-density polyethylene and a low-density polyethylene is preferably used in a blend ratio (a mass ratio) of 1/9 to 9/1, more preferably 2/8 to 8/2, and most preferably 3/7 to 7/3. When the thermoplastic resin layer is formed on the both surfaces of the support, the back side of the support is preferably formed using, for example, the high-density polyethylene or the blend of a high-density polyethylene and a low-density polyethylene. The molecular weight of the polyethylenes is not particularly limited. Preferably, both of the high-density polyethylene and the low-density polyethylene have a melt index of 1.0 to 40 g/10 minute and a high extrudability.

The sheet or film may be subjected to a treatment to impart white reflection thereto. As a method of such a treatment, for example, a method of incorporating a pigment such as titanium oxide into the sheet or film can be mentioned.

The thickness of the support is preferably from 25  $\mu$ m to 300  $\mu$ m, more preferably from 50  $\mu$ m to 260  $\mu$ m, and further preferably from 75  $\mu$ m to 220  $\mu$ m. The support can have any rigidity according to the purpose. When it is used as a support for electrophotographic image-receiving sheet of photographic image quality, the rigidity thereof is preferably near to that in a support for use in color silver halide photography. (Curling Control Layer)

When the support is exposed as it is, there is the case where the heat-sensitive transfer image-receiving sheet is made to curl by moisture and/or temperature in the environment. It is therefore preferable to form a curling control layer on the back side of the support. The curling control layer not only prevents the image-receiving sheet from curling but also has a water-proof function. For the curling control layer, a polyethylene laminate, a polypropylene laminate or the like is used. Specifically, the curling control layer may be formed in a manner similar to those described in, for example, JP-A-61-110135 and JP-A-6-202295. (Writing Layer and Charge Controlling Layer)

For the writing layer and the charge control layer, an inorganic oxide colloid, an ionic polymer, or the like may be used. As the antistatic agent, any antistatic agents including cationic antistatic agents such as a quaternary ammonium salt and polyamine derivative, anionic antistatic agents such as alkyl phosphate, and nonionic antistatic agents such as fatty acid ester may be used. Specifically, the writing layer and the charge control layer may be formed in a manner similar to those described in the specification of Japanese Patent No. 3585585.

The method of producing the heat-sensitive transfer image-receiving sheet according to the present invention is explained below.

The heat-sensitive transfer image-receiving sheet according to the present invention may be prepared by coating each of layers using a usual method such as a roll coating, a bar coating, a gravure coating, or a gravure reverse coating, followed by drying the layers.

Alternatively, the heat-sensitive transfer image-receiving sheet according to the present invention may be also prepared by simultaneous multi-layer coating the receptor layer and the heat insulation layer on the support.

It is known that in the case of producing an image-receiving sheet composed of plural layers having different functions from each other (for example, an air cell layer, heat insulation layer, intermediate layer, and receptor layer) on a support, it may be produced by applying and overlapping each layer one by one or by applying materials prepared in advance by coating a support with each layer, as shown in, for example, JP-A-2004-106283, JP-A-2004-181888 and JP-A-2004-345267. It has been known in photographic industries, on the other hand, that productivity can be greatly improved by applying plural layers simultaneously as a multilayer. For example, there are known methods such as the so-called slide coating (slide coating method) and curtain coating (curtain coating method) as described in, for example, U.S. Pat. Nos. 2,761,791, 2,681,234, 3,508,947, 4,457,256 and 3,993,019; JP-A-63-54975, JP-A-61-278848, JP-A-55-86557, JP-A-52-31727, JP-A-55-142565, JP-A-50-43140, JP-A-63-80872, JP-A-54-54020, JP-A-5-104061, JP-A-5-127305, and JP-B-49-7050; and Edgar B. Gutoff, et al., "Coating and Drying Defects: Troubleshooting Operating Problems", John Wiley & Sons Company, 1995, pp. 101-103.

In the present invention, it has been found that the productivity can be greatly improved and image defects can be remarkably reduced at the same time, by using the above simultaneous multilayer coating for the production of an image-receiving sheet having a multilayer structure.

The plural layers in the present invention are structured using resins as their major components. Coating solutions for forming the respective layers are preferably water-dispersed latexes (latexes in the form of an aqueous dispersion). The solid content by mass of the resin put in a latex state in each layer coating solution is preferably in a range from 5 to 80% and particularly preferably 20 to 60%. The average particle size of the resin contained in the above water-dispersed latex is preferably 5  $\mu\text{m}$  or less and particularly preferably 1  $\mu\text{m}$  or less. The above water-dispersed latex may contain a known additive, such as a surfactant, a dispersant, and a binder resin, according to the need.

In the present invention, it is preferred that a laminate composed of plural layers be formed on a support and solidified just after the forming, according to the method described in U.S. Pat. No. 2,761,791. For example, in the case of solidifying a multilayer structure by using a resin, it is preferable to raise the temperature immediately after the plural layers are formed on the support. Also, in the case where a binder (e.g., a gelatin) which causes gelation at lower temperatures is contained, it is sometimes preferable to drop the temperature immediately after the plural layers are formed on the support.

In the present invention, the coating amount of a coating solution per one layer constituting the multilayer is preferably in a range from 1  $\text{g}/\text{m}^2$  to 500  $\text{g}/\text{m}^2$ . The number of layers in the multilayer structure may be arbitrarily selected from a number of 2 or more. The receptor layer is preferably disposed as a layer most apart from the support.

Next, the heat-sensitive (thermal) transfer sheet (ink sheet) for use in the present invention is explained below.

The ink sheet that is used in combination with the above-mentioned heat-sensitive transfer image-receiving sheet at

the time when a thermal transfer image is formed, is provided with, on a support, a thermal transfer layer containing a diffusion transfer dye (hereinafter, also referred to as "dye layer"). The ink sheet may be arbitrarily selected from any ink sheets. The heat-sensitive transfer sheet is a preferable one, which has three primary color layers containing yellow, magenta or cyan colorants, respectively, in a state that these layers are formed one after another in the direction of the major axis of the heat-sensitive transfer sheet (so that each layer has an area corresponding to the recording surface area of a heat-sensitive transfer image-receiving sheet), and which further has a protective layer transfer section that is provided after the formation of the cyan colorant layer. The content of each dye in the thermal transfer layer (dye layer) is preferably from 10 to 90 mass %, more preferably from 20 to 80 mass %.

The dye layer is applied using a usual method such as a roll coating, a bar coating, a gravure coating, and a gravure reverse coating. A coating amount of the thermal transfer layer in the heat-sensitive transfer sheet (ink sheet) is preferably in the range of 0.1 to 1.0  $\text{g}/\text{m}^2$  (in solid content equivalent), and more preferably in the range of 0.15 to 0.60  $\text{g}/\text{m}^2$ . Hereinafter, the term "coating amount" used herein is expressed by a solid content equivalent value, unless it is indicated differently in particular.

A film thickness of the thermal transfer layer is preferably in the range of 0.1 to 2.0  $\mu\text{m}$ , and more preferably in the range of 0.1 to 1.0  $\mu\text{m}$ .

As a support for the heat-sensitive transfer sheet, use may be made of the same as those for use in the heat-sensitive transfer image-receiving sheet, for example, polyethylene-terephthalate.

A thickness of the support is preferably in the range of 1 to 10  $\mu\text{m}$ , and more preferably in the range of 2 to 10  $\mu\text{m}$ .

With respect to the heat-sensitive transfer sheet, there is a detailed explanation in, for example, JP-A-11-105437. The description in paragraph Nos. 0017 to 0078 of JP-A-11-105437 is incorporated by reference into the specification of the present application.

Next, the image-forming method using the heat-sensitive transfer image-receiving sheet according to the present invention is described.

The present invention is applied to an image formation system in which the foregoing heat-sensitive transfer sheet is superposed on the foregoing heat-sensitive transfer image-receiving sheet so that the thermal transfer layer of the heat-sensitive transfer sheet and the receptor layer of the heat-sensitive transfer image-receiving sheet are brought into face-to-face contact, and thermal energies according to image signals is applied thereto from a thermal head, and continuously produce printed outputs on the thermal transfer image-receiving sheets at intervals of 5 seconds or below between the end of ejection of one sheet printed and the start of ejection of the next sheet printed. Herein, "the interval of 5 seconds or below between the end of ejection of one sheet printed and the start of ejection of the next sheet printed" (i.e. the time interval of 5 seconds or below between the time when ejection of one sheet ends and the time when ejection of the next starts) is preferably defined as the time required for ejection of a L-size print (photo) from an image formation apparatus or system, e.g., a printer. Additionally, it does not matter whether the actual size of output images is smaller or larger than the foregoing size. In other words, the above definition is the criterion for evaluation of the time required for the sheet of standard size.

The time interval between the time when ejection of one sheet ends and the time when ejection of the next starts is preferably from 5 seconds to 0.1 second.

23

As a means for providing heat energy in the thermal transfer, any of the conventionally known providing means may be used. For example, application of a heat energy of about 5 to 100 mJ/mm<sup>2</sup> by controlling recording time in a recording device such as a thermal printer (for example, Video Printer VY-100 (trade name), manufactured by Hitachi, Ltd.), will sufficiently attain the expected result.

Also, the heat-sensitive transfer image-receiving sheet according to the present invention may be used in various applications enabling thermal transfer recording, such as heat-sensitive transfer image-receiving sheets in a form of thin sheets (cut sheets) or rolls; cards; and transmittable type manuscript-making sheets, by optionally selecting the type of support.,

The present invention may be utilized for printers, copying machines and the like, which employ a heat-sensitive transfer recording system.

According to the present invention, it is possible to provide a heat-sensitive transfer image-receiving sheet that is suited for high-speed printing and delivers high-quality images having high densities, no image defects and improved preservability of image and image quality, and a method of forming images.

The present invention will be described in more detail based on the following examples, but the invention is not intended to be limited thereto.

### EXAMPLES

In the following Examples, the terms "part" and "%" are values by mass, unless they are indicated differently in particular.

#### (Preparation of Ink Sheet)

A 4.5  $\mu\text{m}$ -thick polyester film (Lumirror, trade name, manufactured by Toray Industries, Inc.) was used as a substrate film. On the front side of the film, the following adhesive layer (coating amount in a dried-film state: 0.07 g/m<sup>2</sup>) was formed, and further the yellow, magenta, and cyan compositions described below were respectively applied as monochromatic (single color) layers (coating amount in a dried-film state: 1 g/m<sup>2</sup>).

#### <Composition solution for adhesive layer>

Polyvinylpyrrolidone resin  
(trade name: K-90, manufactured by ISP Co., Ltd.)

5 parts by mass

Methyl ethyl ketone  
Isopropyl alcohol

47.5 parts by mass  
47.5 parts by mass

#### <Composition solution for dye layer>

##### Yellow composition

Dye (7)-1  
Dye (8)-1  
Polyester 1  
Methyl ethyl ketone/toluene (1/1, at mass ratio)  
Magenta composition

2.5 parts by mass  
2.0 parts by mass  
4.5 parts by mass  
90 parts by mass

Dye (9)-1  
Dye (10)-1  
Dye (11)-1  
Polyester 1  
Methyl ethyl ketone/toluene (1/1, at mass ratio)  
Cyan composition

1.0 parts by mass  
1.0 parts by mass  
2.5 parts by mass  
4.5 parts by mass  
90 parts by mass

Dye (12)-1  
Dye (13)-1  
Polyester 1

2.5 parts by mass  
2.5 parts by mass  
4.5 parts by mass

24  
-continued

Methyl ethyl ketone/toluene (1/1, at mass ratio) 90 parts by mass

(7)-1



25

-continued

(12-1)



The above-described polyester 1 has the composition set forth below.

(Polyester 1)

Polyester having a number-average molecular weight of 2000, that was obtained by polymerizing the following molar ratio of acid and diol components as described below.

|                   |    |
|-------------------|----|
| Isophthalic acid  | 5  |
| Terephthalic acid | 45 |
| Ethyleneglycol    | 5  |
| Diethyleneglycol  | 45 |

Further, a heat-resistant sliding layer (coating amount in a dried-film state: 1 g/m<sup>2</sup>) was formed on the back side of the film, thereby forming an ink sheet.

<Composition solution for heat-resistant sliding layer>

|                                                                                                          |                    |
|----------------------------------------------------------------------------------------------------------|--------------------|
| Polyvinylbutyral resin<br>(S-LEC BX-1, (trade name) manufactured<br>by Sekisui Chemical)                 | 13.6 parts by mass |
| Polyisocyanate hardening agent<br>(Takenate D218, (trade name) manufactured<br>by Takeda Pharmaceutical) | 0.6 parts by mass  |
| Phosphoric ester<br>(PLY-SURFA208S, (trade name) manufactured<br>by DAI-ICHI KOGYOU SEIYAKU)             | 0.8 parts by mass  |
| Methyl ethyl ketone                                                                                      | 42.5 parts by mass |
| Toluene                                                                                                  | 42.5 parts by mass |

(Preparation of Image-Receiving Sheets)

(Sample 101 for Comparison)

Preparation of Image-Receiving Sheet 101

Synthetic paper (trade name: Yupo FPG 200, manufactured by Yupo Corporation, thickness: 200 µm) was used as the support, and a receptor layer having the following composition was applied to one surface of this support. The applica-

26

tion was carried out such that the amount of the receptor layer was 4.0 g/m<sup>2</sup>, and the layer was dried at 110° C. for 30 seconds.

5

Coating solution for receptor layer 1  
(Composition)

|                                                                                                    |                   |
|----------------------------------------------------------------------------------------------------|-------------------|
| Polyester resin<br>(Trade name: Vylon 200, manufactured by<br>Toyobo Co., Ltd.)                    | 100 parts by mass |
| Amino-modified silicone<br>(X-22-343 (trade name) manufactured by<br>Shin-Etsu Chemical Co., Ltd.) | 3 parts by mass   |
| Epoxy-modified silicone<br>(KF-393 (trade name) manufactured by<br>Shin-Etsu Chemical Co., Ltd.)   | 3 parts by mass   |
| Toluene/methyl ethyl ketone (1/1, at mass ratio)<br>(Coating amount) 20 ml/m <sup>2</sup>          | 500 parts by mass |

(13-1)

(Sample 102 According to the Present Invention)

Preparation of Image-Receiving Sheet 102

(Preparation of Support)

A pulp slurry was prepared from 50 parts by mass of hardwood kraft pulp (LBKP) of acacia origin and 50 parts by mass of hardwood kraft pulp (LBKP) of aspen origin, by beating these pulps by means of a disk refiner until Canadian standard freeness reached to 300 ml.

To the pulp slurry thus prepared were added, on a pulp basis, 1.3 mass % of modified cationic starch (CAT0304L, trade name, manufactured by Nippon NSC), 0.15 mass % of anionic polyacrylamide (DA4104, trade name, manufactured by Seiko PMC Corporation), 0.29 mass % of an alkylketene dimer (SIZEPINE K, trade name, manufactured by Arakawa Chemical Industries, Ltd.), 0.29 mass % of epoxidated behenic acid amide, and 0.32 mass % of polyamide polyamine epichlorohydrin (ARAFIX 100, trade name, manufactured by Arakawa Chemical Industries, Ltd.), and thereafter 0.12 mass % of a defoaming agent was further added.

The resulting pulp slurry was made into paper by use of a fourdrinier paper machine. In a process of drying in which the felt side of web was pressed against a drum dryer cylinder via a dryer canvas, the web thus formed was dried under a condition that the tensile strength of the dryer canvas was adjusted to 1.6 kg/cm. Then, each side of the raw paper thus made was coated with 1 g/m<sup>2</sup> of polyvinyl alcohol (KL-118, trade name, manufactured by Kuraray Co., Ltd.) with a size press, then, dried and further subjected to calendering treatment. Therein, the papermaking was performed so that the raw paper had a grammage (basis weight) of 157 g/m<sup>2</sup>, and the raw paper (base paper) having a thickness of 160 µm was obtained.

The wire side (back side) of the base paper obtained was subjected to corona discharge treatment, and thereto a resin composition, in which a high-density polyethylene having an MFR (which stands for a melt flow rate, and hereinafter has the same meaning) of 16.0 g/10 min and a density of 0.96 g/cm<sup>3</sup> (containing 250 ppm of hydrotalcite (DHT-4A (trade name), manufactured by Kyowa Chemical Industry Co., Ltd.) and 200 ppm of a secondary oxidation inhibitor (tris(2,4-di-t-butylphenyl)phosphite, Irugaphos 168 (trade name), manufactured by Ciba Specialty Chemicals)) and a low-density polyethylene having an MFR of 4.0 g/10 min and a density of 0.93 g/cm<sup>3</sup> were mixed at a ratio of 75 to 25 by mass, was applied so as to have a thickness of 21 g/m<sup>2</sup>, by means of a melt extruder, thereby forming a thermoplastic resin layer with a mat surface. (The side to which this thermoplastic resin

layer was provided is hereinafter referred to as "back side". The thermoplastic resin layer at the back side was further subjected to corona discharge treatment, and then coated with a dispersion prepared by dispersing into water a 1:2 mixture (by mass) of aluminum oxide (ALUMINASOL 100, trade name, manufactured by Nissan Chemical Industries, Ltd.) and silicon dioxide (SNOWTEX O, trade name, manufactured by Nissan Chemical Industries, Ltd.), as an antistatic agent, so that the coating had a dry mass of 0.2 g/m<sup>2</sup>. Subsequently, the front surface (front side) of the base paper was subjected to corona discharge treatment, and then coated with 27 g/m<sup>2</sup> of a low-density polyethylene having an MFR of 4.0 g/10 min and a density of 0.93 g/m<sup>3</sup> and containing 10 mass % of titanium oxide, by means of a melt extruder, thereby forming a thermoplastic resin layer with a specular surface.

(Preparation of Emulsion)

An emulsified dispersion A was prepared in the following manner. A compound A-6 was dissolved in a mixture of 42 g of a high-boiling solvent (Solv-1) and 20 ml of ethyl acetate, and the resulting solution was emulsified and dispersed in 250 g of a 20 mass % aqueous gelatin solution containing 1 g of sodium dodecylbenzenesulfonate by means of a high-speed stirring emulsification machine (dissolver). Thereto, water was added to prepare 380 g of an emulsified dispersion A.

Therein, the addition amount of compound A-6 was adjusted so that the compound would be contained in an amount of 30 mol % in the emulsified dispersion A.



Coating solutions described below were given to the support prepared in the foregoing manner so as to form a multi-layer structure having an subbing layer, a heat insulation layer, and a receptor layer, by simultaneous multi-layer coating, in increasing order of distance from the support, thereby

making an image-receiving sheet. Compositions and application amounts of the coating solutions used herein are shown below.

5

Coating solution for subbing layer  
(Composition)

|    |                                                                                                                                                                                                            |                                      |
|----|------------------------------------------------------------------------------------------------------------------------------------------------------------------------------------------------------------|--------------------------------------|
| 10 | Styrene-butadiene latex (SR103 (trade name), manufactured by Nippon A & L Inc.)<br>6% Aqueous solution of polyvinyl alcohol (PVA)<br>NaOH for adjusting pH to 7.5<br>(Coating amount) 11 ml/m <sup>2</sup> | 60 parts by mass<br>40 parts by mass |
| 15 | Coating solution for heat insulation layer<br>(Composition)                                                                                                                                                |                                      |

|    |                                                                                                                        |                                      |
|----|------------------------------------------------------------------------------------------------------------------------|--------------------------------------|
| 15 | Hollow latex polymer (MH5055 (trade name), manufactured by Zeon Corporation)<br>10% Gelatin aqueous solution           | 60 parts by mass                     |
| 20 | Emulsified dispersion A prepared in the above<br>NaOH for adjusting pH to 7.8<br>(Coating amount) 38 ml/m <sup>2</sup> | 20 parts by mass<br>20 parts by mass |
| 20 | Coating solution for receptor layer 2<br>(Composition)                                                                 |                                      |
| 25 |                                                                                                                        |                                      |

|    |                                                                                                                                                    |                                     |
|----|----------------------------------------------------------------------------------------------------------------------------------------------------|-------------------------------------|
| 25 | Vinyl chloride-series latex polymer (VINYBLAN 900, trade name, manufactured by Nissin Chemical Industry Co., Ltd.)                                 | 50 parts by mass                    |
| 30 | Vinyl chloride-series latex polymer (VINYBLAN 276, trade name, manufactured by Nissin Chemical Industry Co., Ltd.)<br>10% Gelatin aqueous solution | 20 parts by mass                    |
| 30 | Emulsified dispersion A prepared in the above<br>Microcrystalline wax (EMUSTAR-042X (trade name), manufactured by Nippon Seiro Co., Ltd.)          | 10 parts by mass                    |
| 35 | Hardener (VS-7)<br>Water<br>NaOH for adjusting pH to 7.4<br>(Coating amount) 18 ml/m <sup>2</sup>                                                  | 0.2 part by mass<br>5 parts by mass |

35

The hardener (VS-7) used herein was the following compound.



(Image-Receiving Sheets 103 to 114)

Image-receiving sheets 103 to 108 were prepared in the same manner as the image-receiving sheet 102, except that the vinyl chloride latex polymer was changed to the compounds shown in Table 1, respectively.

Further, image-receiving sheets 109 to 114 were prepared in the same manner as the image-receiving sheets 103 to 108, respectively, except that the heat insulation layers of the image-receiving sheets 103 to 108 were omitted.

TABLE 1

| No. | Heat<br>sample<br>insulation | Image-receiving layer |                                                                                      |                         |                     |
|-----|------------------------------|-----------------------|--------------------------------------------------------------------------------------|-------------------------|---------------------|
|     |                              | layer                 | Kind of polymer                                                                      | Composition of polymer  |                     |
| 103 | Present                      |                       | VYLONAL MD1100<br>(trade name, manufactured by Toyobo Co., Ltd.)                     | Polyester               | Comparative example |
| 104 | Present                      |                       | VYLONAL MD1480<br>(trade name, manufactured by Toyobo Co., Ltd.)                     | Polyester               | Comparative example |
| 105 | Present                      |                       | Saran latex L536B<br>(trade name, manufactured by Asahi Kasei Chemicals Corporation) | Polyvinylidene chloride | Comparative example |
| 106 | Present                      |                       | VINYBLAN 430                                                                         | Polyvinyl chloride      | This                |

TABLE 1-continued

| No. | Heat<br>Sample insulation | Image-receiving layer                                                                |                                        |                        |         |
|-----|---------------------------|--------------------------------------------------------------------------------------|----------------------------------------|------------------------|---------|
|     |                           | layer                                                                                | Kind of polymer                        | Composition of polymer | Remarks |
| 107 | Present                   | VINYBLAN 601<br>(trade name, manufactured by Nissin Chemical Industry Co., Ltd.)     | Vinyl chloride-vinyl acetate copolymer | This invention         |         |
| 108 | Present                   | VINYBLAN 609<br>(trade name, manufactured by Nissin Chemical Industry Co., Ltd.)     | Vinyl chloride-acryl copolymer         | This invention         |         |
| 109 | Absent                    | VYLONAL MD1100<br>(trade name, manufactured by Toyobo Co., Ltd.)                     | Polyester                              | Comparative example    |         |
| 110 | Absent                    | VYLONAL MD1480<br>(trade name, manufactured by Toyobo Co., Ltd.)                     | Polyester                              | Comparative example    |         |
| 111 | Absent                    | Saran latex L536B<br>(trade name, manufactured by Asahi Kasei Chemicals Corporation) | Polyvinylidene chloride                | Comparative example    |         |
| 112 | Absent                    | VINYBLAN 430<br>(trade name, manufactured by Nissin Chemical Industry Co., Ltd.)     | Polyvinyl chloride                     | Comparative example    |         |
| 113 | Absent                    | VINYBLAN 601<br>(trade name, manufactured by Nissin Chemical Industry Co., Ltd.)     | Vinyl chloride-vinyl acetate copolymer | Comparative example    |         |
| 114 | Absent                    | VINYBLAN 609<br>(trade name, manufactured by Nissin Chemical Industry Co., Ltd.)     | Vinyl chloride-acryl copolymer         | Comparative example    |         |

## (Image Formation 1 for Comparison)

The ink sheet and each of the image-receiving sheets 101 to 114 were both worked to be made loadable, and from a dye sublimation printer ASK1500 (made by Fuji Photo Film Co., Ltd.) in a high-speed printing mode outputs of a black solid image (L-size) were produced continuously on 10 sheets per each image-receiving sheet. Herein, the time interval between the time when ejection of one sheet ends and the time when ejection of the next starts was 12 seconds.

## (Dmax Evaluation)

The visual density of the black image output produced on each second sheet under the foregoing condition was measured with a Photographic Densitometer (made by X-Rite Incorporated).

The results obtained are shown in Table 2. As can be seen from Table 2, in the image formation system having the continuous output time of 12 seconds the image-receiving sheets 102 and 106 to 108 according to the present invention were unable to attain so higher Dmax than comparative image-receiving sheets.

## (Image Formation 2 According to the Present Invention)

The printer disclosed in FIG. 6 of JP-A-5-278247 was set so that the intervals of outputs in continuous printing would be 5 seconds, and the ink sheet and each of the image-receiving sheets 101 to 114 were both worked to be made loadable, and from the printer in a high-speed printing mode outputs of a black solid image were produced continuously on 10 sheets per each image-receiving sheet. Herein, the time interval between the time when ejection of one sheet ends and the time when ejection of the next starts was 4.8 seconds.

## (Dmax Evaluation)

The visual density of the black image output produced on each second sheet under the foregoing condition was measured with a Photographic Densitometer (made by X-Rite Incorporated).

The results obtained are shown in Table 3. As can be seen from Table 3, in the image formation system having the continuous output time of 5 seconds or below the image-receiving sheets 102 and 106 to 108 according to the present invention were able to attain significantly higher Dmax than comparative image-receiving sheets.

TABLE 2

| Sample No. | Dmax | Remarks             |
|------------|------|---------------------|
| 101        | 1.85 | Comparative example |
| 102        | 1.90 | This invention      |
| 103        | 1.62 | Comparative example |
| 104        | 1.67 | Comparative example |
| 105        | 1.48 | Comparative example |
| 106        | 1.81 | This invention      |
| 107        | 1.83 | This invention      |
| 108        | 1.79 | This invention      |
| 109        | 1.58 | Comparative example |
| 110        | 1.62 | Comparative example |
| 111        | 1.48 | Comparative example |
| 112        | 1.59 | Comparative example |
| 113        | 1.55 | Comparative example |
| 114        | 1.49 | Comparative example |

TABLE 3

| Sample No. | Dmax | Remarks             |
|------------|------|---------------------|
| 55         | 101  | Comparative example |
|            | 102  | This invention      |
|            | 103  | Comparative example |
|            | 104  | Comparative example |
|            | 105  | Comparative example |
|            | 106  | This invention      |
|            | 107  | This invention      |
| 60         | 108  | This invention      |
|            | 109  | Comparative example |
|            | 110  | Comparative example |
|            | 111  | Comparative example |
|            | 112  | Comparative example |
|            | 113  | Comparative example |
| 65         | 114  | Comparative example |

## 31

Having described our invention as related to the present embodiments, it is our intention that the invention not be limited by any of the details of the description, unless otherwise specified, but rather be construed broadly within its spirit and scope as set out in the accompanying claims.

What we claim is:

1. A method of forming an image,

which method uses:

a heat-sensitive transfer image-receiving sheet which has,

on a support, at least one receptor layer containing a latex polymer comprising repeating units of vinyl chloride component and at least one heat insulation layer containing hollow polymeric particles, and

a heat-sensitive transfer sheet which has a transfer layer containing a thermally transferable color material;

which method comprises the steps of:

superposing the heat-sensitive transfer image-receiving sheet upon the heat-sensitive transfer sheet, so that the transfer layer of the heat-sensitive transfer sheet and the receptor layer of the heat-sensitive transfer image-receiving sheet are brought into face-to-face contact with each other, and

applying a thermal energy according to image signals thereto from a thermal head, and

continuously producing printed outputs on the thermal transfer image-receiving sheets at intervals of 5 seconds or below between the end of ejection of one sheet printed and the start of ejection of the next sheet printed.

2. The method of forming an image as claimed in claim 1, wherein the heat insulation layer does not contain any resins having poor resistance to an organic solvent other than the hollow polymeric particles.

## 32

3. The method of forming an image as claimed in claim 1, wherein at least one of the receptor layer and the heat insulation layer further contains a water-soluble polymer.

4. The method of forming an image as claimed in claim 1, wherein at least one of the receptor layer containing the water-soluble polymer and the heat insulation layer containing the water-soluble polymer further contains a compound capable of forming crosslinks between molecules of the water-soluble polymer and the compound brings a part or all of the water-soluble polymer molecules into being crosslinked.

5. The method of forming an image as claimed in claim 1, wherein the latex polymer is a vinyl chloride-acryl copolymer.

6. The method of forming an image as claimed in claim 1, wherein the receptor layer contains at least two latex polymers which are vinyl chloride-acryl copolymers.

7. The method of forming an image as claimed in claim 1, wherein the particle size of the hollow polymeric particles is 0.1 to 20  $\mu\text{m}$ , and the hollow polymeric particles are non-foaming type hollow polymeric particles which are formed of a styrene/acryl resin.

8. The method of forming an image as claimed in claim 1, wherein the heat insulation layer comprises a gelatin.

9. The method of forming an image as claimed in claim 1, wherein an undercoat layer is provided between the heat insulation layer and the support, the heat insulation layer is superposed on the undercoat layer, and the undercoat layer and any one of the layers thereon comprise a latex polymer.

10. The method of forming an image as claimed in claim 1, wherein an emulsified dispersion is incorporated in the receptor layer or the heat insulation layer.

\* \* \* \* \*